

# United States Patent Office

2,875,089

Patented Feb. 24, 1959

1

2,875,089

## PROCESS FOR THE OPTICAL BRIGHTENING OF MATERIALS OF POLYESTERS

Franz Ackermann, Binningen, and Adolf Emil Siegrist, Basel, Switzerland, assignors to Ciba Limited, Basel, Switzerland, a Swiss firm

No Drawing. Application February 6, 1956  
Serial No. 563,446

Claims priority, application Switzerland February 15, 1955

6 Claims. (Cl. 117—33.5)

This invention is based on the observation that materials of polyesters, especially polyester fibers, can be optically brightened when such a material is treated with a non-quaternary compound having no dyestuff character, which is colorless or only slightly colored, contains no acid salt-forming or water-solubilizing group, which in solution or on a substratum fluoresces green-blue to violet in daylight or ultra-violet light and which contains two five-membered heterocyclic rings, each of which consists of two adjacent carbon atoms which are at the same time ring members of a benzene ring, a nitrogen atom attached to one of the two mentioned carbon atoms, a hetero atom having an atomic number of at least 7 and at most 8, viz. an oxygen, or nitrogen atom attached to the other of the two mentioned carbon atoms and a carbon atom attached to both hetero atoms, the two latter carbon atoms of the two heterocyclic rings being attached together by way of an ethylene bridge.

The material to be improved by the use of the present process can exist in any stage of processing, it being obviously advantageous to treat it in the described manner at a stage when all other treatments have been completed which would have the effect of removing again the agent used according to the invention or would have an unfavorable effect upon it. The agents used can for example be added to the material to be improved either before or during the shaping thereof. Thus they can be added to the moulding mass to be used in the manufacture of foils or shaped bodies or can be dissolved or finely distributed in a spinning mass before the spinning thereof.

The present process has proved to be of especial advantage for the improvement of textile fibers of the specified constitution. As fibers to be treated, such of polyesters of terephthalic acid are especially concerned. Staple fibers or also monofilaments can be used, for example the products obtainable under the names "Dacron" and "Terylene."

The compounds used according to this invention for the improvement of the specified materials must satisfy the requirements set forth in their above-description. They must contain no acid salt-forming or water-solubilizing groups, that is to say no sulfonic acid or carboxylic acid groups. Moreover, they must at most be only slightly colored and must have no dyestuff character, i. e. they should not dye the material under treatment when applied in the customary concentrations. The compounds have as a rule basic character and can be used in the present process either as free bases or in the form of salts which are capable of the formation of the free bases. As above specified, however, the use is excluded from the present process of the quaternary salts obtainable from these compounds (imidazolium, oxazolium or thiazolium compounds).

As stated above the compounds used in the improvement process of this invention contain two 5-membered heterocyclic-rings and each of these rings, which as regards chemical constitution are comprised within the

2

definition azole rings, possesses a structure which corresponds to one or other of the following formula

(1)



5

and

10 (2)



15

In both rings the two adjacent carbon atoms are at the same time ring members of a benzene ring which may contain further substituents. Moreover, the two rings are attached together through the carbon atom between the

20

two hetero atoms by way of an ethylene bridge.

Accordingly, in the present process compounds are used of the formula

(3)



25

in which A indicates a benzene radical condensed with the hetero ring as shown by the valence bonds, B is an oxygen atom or the group



30

in which R1 indicates an alkyl radical, an aralkyl radical or a dialkylaminoalkyl radical and D is an oxygen atom or the group



40

in which R2 indicates an alkyl radical, an aralkyl radical, a dialkylaminoalkyl radical, a hydroxyalkyl radical or a hydrogen atom.

45

As especially advantageous have proved those compounds of the Formula 3 of which the ring members B and D are nitrogen atoms of which each is also further attached to a low molecular alkyl radical, for example such a radical containing at most six carbon atoms, but preferably an ethyl or methyl group.

50

Since the double bonds of the radical A of the above-mentioned general formulae are in conjugation with the double bond of the heterocyclic ring, by suitable substitution of this radical an increase of the fluorescence can also be attained. As substituents in the radical A there are concerned alkyl, alkoxy, alkylamino or acylamino groups or halogen atoms.

Thus, for example, valuable results can also be achieved with the compounds of the formula

(4)



60

In this formula A1 indicates a benzene radical condensed in the specified manner with the imidazole ring, preferably a benzene radical which can be substituted by an alkyl group, for example a methyl group, and R3 is a hydrogen atom, an alkyl group, a hydroxyalkyl group, a dialkylaminoalkyl group or an aralkyl radical. Especially favorable results are obtained as a rule with those

$\alpha;\beta$ -di-[benzoxazolyl-(2)]-ethylenes of the Formula 3 whose benzene radicals A are substituted by low molecular alkyl groups, particularly methyl groups which are preferably in the 5-positions of the benzoxazole radicals.

The compounds to be used in the present process are known in large numbers and others can be prepared by customary methods known per se.

If it is a question of improving textile fibers by the present process which can exist as staple fibers or monofilaments, in the crude state or in the form of yarns or fabrics, this operation is conducted with advantage in an aqueous medium in which the compounds to be used are dissolved or suspended. If desired dispersing agents can be added in the treatment, for example, soaps, polyglycol ethers of fatty alcohols or fatty amines, cellulose sulfite waste liquor or condensation products with formaldehyde of naphthalene sulfonic acids which may be alkylated.

It is of particular advantage, especially when the treatment of the fibers is exclusively for the purpose of improving the optical properties, to work in neutral, weakly alkaline or acid baths. It is likewise of advantage if the treatment takes place at elevated temperature, for example at the boiling temperature of the bath or in the neighborhood thereof (about 90° C.). It is surprising that the compounds of the composition set forth above possess a good affinity for the fibers and can be fixed thereon in a similar manner to dyestuffs. In this connection it may be remarked that in the case of these synthetic fibers many optical improving and brightening agents which are of good applicability for other fiber materials, cannot be used for the reason that in this case they cannot be fixed on the fiber or do not give rise to the desired effect. The fastness to light of the materials treated according to the present process is also good, the effect persisting even after long exposure to light.

The quantity of the improving agent to be used, calculated on the material to be treated, can vary within wide limits. Even with very small quantities, in some cases, for example, of 0.01 percent, a distinct and permanent effect can be attained. Although quantities of more than about 3 percent are in general not disadvantageous, they offer no advantages compared with the normal quantities.

As indicated above, the present process can advantageously be combined with other processing methods. Thus the compounds to be used according to the present invention can also be applied as follows:

(a) In admixture with dyestuffs or as additions to dyebaths or printing, discharge or reserve pastes. Further also for the after-treatment of dyeings, prints or discharge prints, especially in the soaping process. Thus, for example, the polyester fibers can be simultaneously dyed and improved as regards optical properties if they are treated according to the present process, advantageously in the presence of a dispersing agent and dyed by the dispersion method, using as dyestuffs colored compounds which possess the anthracene structure and which in addition contain at least one nuclear-bound oxo group, at least one hydroxyl group or a non-water-solubilizing, sulfur-containing substituent and in which the number of any basic, nitrogen-containing groups present is at most equal to the number of the hydroxyl groups and sulfur-containing substituents. As examples of such compounds may be mentioned 1-hydroxy-anthraquinone, 1-amino-4:5:8-trihydroxy-anthraquinone and 1-amino-4-hydroxyanthraquinone.

(b) In admixture with chemical bleaching agents or as additions to bleaching baths.

(c) In admixture with finishing agents such as starch or synthetic finishes. The compounds to be used according to the invention can for example also be added to the baths used for the production of a crease-proof finish.

(d) In combination with washing agents: The washing agents and brightening agents can be separately added to the washing baths to be used. It is also advantageous to use washing agents which contain brightening agents admixed therewith. As washing agents are suitable for example, soaps, salts of sulfonated washing agents, as for example, of sulfonated benzimidazoles substituted on the 2-carbon atom by higher alkyl residues, also salts of monocarboxylic acid esters of 4-sulfophthalic acid with higher fatty alcohols or salts of fatty alcohol sulfonates, alkylaryl sulfonic acids or condensation products of higher fatty acids with aliphatic hydroxy- or amino-sulfonic acids. Non-ionic washing agents can also be used, for example polyglycol ethers which are derived from ethylene oxide and higher fatty alcohols, alkyl phenols or fatty amines.

The washing agents of the above specified type can also contain the customary washing agent additions, such as alkali metal carbonates, phosphates, pyrophosphates, polyphosphates, metaphosphates, silicates, perborates or percarbonates, so long as the brightening agents are compatible with such additions. It is also possible to prepare washing agents which consist solely or for the most part of inorganic compounds of cleansing effect and the brightening agents. The production of the mixtures of the washing agents and optical brightening agents takes place in a simple manner by mixing and/or grinding of the components together. In this case it may be of advantage to use one or the other component in the dissolved or molten condition for the purpose of facilitating distribution.

In general a small addition of the optical improving agents to the washing agents suffices. There are concerned, for example, quantities of 0.1 to 5 percent calculated on the washing agent. Also smaller quantities, for example, 0.01 percent or even less can be added. Also mixtures with other known brightening agents can be used. The washing agents are used in the customary washing processes. In this manner materials to be cleansed can be simultaneously washed and brightened.

When the present process is combined with other treatment or improvement methods, for example those set forth above under (a) to (d), the combined treatment advantageously takes place with the aid of suitably constituted preparations. These stable preparations are characterized by a content of compounds of the type specified above, especially derivatives of oxazole, and also further textile treating agents, for example dyestuffs, chemical bleaching agents, finishing agents or especially washing agents.

Further valuable preparations which are primarily suited for the improvement of polyester fiber as regards optical properties alone, that is to say without additional treatment according to (a) to (d), are distinguished by the fact that they contain in addition to the compounds of the composition initially described above also acid-reacting, preferably solid substances. As examples of such substances may be mentioned sodium bisulfate, tartaric acid and urea nitrate.

The following examples illustrate the invention, the parts and percentages being by weight unless otherwise stated:

#### Example 1

Polyester fabrics are treated for 20 minutes at 80-100° C. in a bath ratio 1:40 with 0.02 percent of  $\alpha;\beta$ -di-[benzoxazolyl-(2)]-ethylene of the formula



in a bath which contains per liter 1 gram of disodium sulfate and 1 gram of the sodium salt of 2-heptadecyl-N-benzylbenzimidazolyl-disulfonic acid. The material is

then rinsed and dried. The resulting fabric has a higher white content than the untreated material. If instead of 1 gram of disodium sulfate, 1 gram of 85 percent formic acid is used, a similar effect is attained.

*Example 2*

The process is conducted as described in Example 1 but there is used instead of 0.02 percent of  $\alpha:\beta$ -di-[benzoxazyl-(2)]-ethylene 0.2 percent of  $\alpha$ -[N-hydroxyethylbenzimidazyl-(2)]- $\beta$ -[N-methylbenzimidazyl-(2)]-ethylene of the formula



The fabric appears brighter than the untreated material.

Similar effects are obtained with the compounds of the following formulae



(prepared from fumaric acid dibenzimidazole or from maleic acid dibenzimidazole and benzyl chloride)



*Example 3*

30 parts of  $\alpha:\beta$ -di-[N-methylbenzimidazyl-(2)]-ethylene are ground to a fine, homogeneous powder in a suitable mixing and grinding apparatus with 60 parts of sodium bisulfate and 910 parts of a condensation product from naphthalene sulfonic acid and formaldehyde.

Polyester fibers, for example "Terylene," which have been treated in a bath ratio of 1:30 for 30 minutes at 80-100° C. with 2 percent of this powder in a bath which contains per liter 1-2 cc. of ammonia, then rinsed and dried, possess a brighter appearance than the untreated material.

If the 60 grams of sodium bisulfate are replaced by 60 grams of a condensation product from naphthalene sulfonic acid and formaldehyde or 60 grams of urea nitrate or 60 grams of tartaric acid, a product with similar properties is obtained.

Similar effects are obtained with  $\alpha:\beta$ -di-[N-ethylbenzimidazyl-(2)]-ethylene.

*Example 4*

50 parts of  $\alpha:\beta$ -di-[N-methylbenzimidazyl-(2)]-ethylene are ground to a fine, homogeneous powder with 950

parts of tartaric acid. Polyester fibers, for example "Dacron" which are treated in a bath ratio of 1:40 for 30 minutes at 90-95° C. with 1 percent of the powder in a bath which contains per liter 1-2 cc. of ammonia and 1 gram of the sodium salt of 2-heptadecyl-N-benzylbenzimidazyl-disulfonic acid, then rinsed and dried, possess a brighter appearance than the untreated material.

By using instead of 1 gram of the above preparation, 1 gram of a powder which contains instead of the tartaric acid, sodium bisulfate or urea nitrate or another suitable solid substance soluble in water with an acid reaction, the resulting fabric has a similar effect.

15

A soap is produced which contains 0.3 percent of  $\alpha:\beta$ -di-[5-methylbenzoxazolyl-(2)]-ethylene.

Polyester fibers, for example "Terylene," which have been washed in the usual way with this soap, have a brighter appearance than material which is only washed with soap.

A similar effect is obtained when there is added per liter of wash liquor 0.5 gram of active chlorine in the form of sodium hypochlorite.

25 Instead of the soap a washing material can be used of the following composition

33.3 percent of soap

11.0 percent of anhydrous sodium carbonate

14.0 percent of sodium pyrophosphate

7.0 percent of sodium perborate

3.0 percent of magnesium silicate

0.3 percent of  $\alpha:\beta$ -di-[5-methylbenzoxazolyl-(2)]-ethylene

35 31.4 percent of water

or also synthetic washing agents.

*Example 5*

12 parts of  $\alpha:\beta$ -di-[5-methylbenzoxazolyl-(2)]-ethylene are worked up to a finely dispersed paste with 12 parts of an addition product from about 30 mols of ethylene oxide to a mixture of saturated fatty alcohols most of which have 18 carbon atoms and 76 parts of water.

Polyester fibers, for example "Dacron," which are treated in a bath ratio of 1:30 for 30 minutes at 60-100° C. with 0.2 percent of this paste in a bath which contains per liter 1 cc. of ammonia, then rinsed and dried, possess a brighter appearance than the untreated material.

50 Instead of the above described addition product, other dispersion agents can also be used, for example a condensation product from naphthalene sulfonic acid and formaldehyde.

The  $\alpha:\beta$ -di-[5-methylbenzoxazolyl-(2)]-ethylene may be prepared as follows:

76 parts of fumaric acid dichloride are added dropwise to a solution of 123 parts of 1-amino-2-hydroxy-5-methylbenzene in 1200 parts of chlorobenzene with stirring and exclusion of air at 125-130° C. in the course of one hour, and the mixture is then maintained at a gentle boil for 6 hours. The resulting yellowish condensation product of the formula



is filtered off, washed with chlorobenzene, alcohol and water and dried.

30 parts of the acylamino compound of the above formula are added to a melt of 10 parts of ethylene-glycol and 150 parts of zinc chloride at 155-160° C. in the course of about 1/4 hour, and the mixture is then stirred for 10 hours at 160-165° C. 600 parts of cold water are

then added dropwise, the temperature being allowed to drop. Concentrated hydrochloric acid is then added until the reaction is acid. The mixture is stirred for another hour at about 60° C., the separated product is filtered off, washed with water until the filtrate shows a neutral reaction and, if necessary, is crystallized from dioxane. There is obtained  $\alpha:\beta$ -di-[5-methyl-benzoxazolyl-(2)]-ethylene in the form of pale crystals which melt at 292° C. The solution in dioxane exhibits a bluish fluorescence.

*Example 7*

A mixed fabric from polyester fibers, for example "Terylene" and wool is treated in a bath ratio 1:50 for 30 minutes at 60-90° C. with 2 percent of the preparation obtained according to Example 3, in a bath containing 1 gram of ammonia per liter.

The resulting fabric has a higher white content than the untreated material.

A similar effect is obtained in the case of a fabric consisting of polyester fibers, for example "Terylene," and 20 polyamide fibers, for example "Perlon."

*Example 8*

100 parts of polyester fabric, for example "Terylene," are treated for one hour at 60-90° C. in a bath of the 25 following composition:

3 liters of water  
6 grams of 85 percent formic acid

6 grams of sodium chlorite

0.7 gram of the product described in Example 6, rinsed 30 and dried

The material thus treated has a higher white content than a material treated without the addition of the di-benzoxazole compound.

A similar effect is obtained where 15 cc. of 40% peracetic acid are used instead of the formic acid and sodium chlorite.

*Example 9*

"Terylene" fabric is dyed for one hour at 90-95° C. 40 in a bath which (calculated on the fabric) contains:

2% 1:4-dimethylamino-anthraquinone and

4%  $\alpha:\beta$ -di-[N-methyl-benzimidazolyl-(2)]-ethylene

The goods to liquor ratio is 1:40. After being rinsed 45 and dried the fabric so treated has a pure greenish blue and bluish fluorescent shade.

A fabric dyed in the same manner but without the addition of the di-imidazole compound is less pure in shade and does not fluoresce.

*Example 10*

"Terylene" fabric is treated at 80-90° C. in a finishing bath of the following composition:

1 liter water  
20 grams potato starch

1 cc. ammonia 24%

0.5 gram of the product described in the first paragraph of Example 6

After squeezing and drying the material thus finished has a brighter appearance than material which has been finished only with starch.

What is claimed is:

1. A process for the optical brightening of materials of polyesters which comprises treating the material with a non-quaternary compound which is free from acid salt-forming, water solubilizing groups and groups imparting dyestuff character, which in solution fluoresces green-blue to violet and which corresponds to the formula



in which A is a monocyclic aromatic radical condensed in the manner indicated by the valence bonds with the oxazole ring.

5. A process for the optical brightening of polyester fibers which comprises applying to said fibers in a finely dispersed state the optical brightening agent of the formula



10. 3. A process for the optical brightening of polyester fibers which comprises applying to said fibers in the presence of a dispersing agent the optical brightening agent of the formula



15. 4. A process for the optical brightening of polyester fibers which comprises applying to said fibers in the presence of a washing agent the optical brightening agent of the formula



20. 5. A composition of matter substantially consisting of a polyester and having incorporated in it a small quantity of a non-quaternary compound which is free from acid salt-forming, water solubilizing groups and groups imparting dyestuff character, which in solution fluoresces green-blue to violet and which corresponds to the formula



25. in which A is monocyclic aromatic radical condensed in the manner indicated by the valence bonds with the oxazole ring.

55. 6. A composition of matter substantially consisting of polyester fibers having incorporated a small quantity of the optical brightening agent of the formula



**References Cited in the file of this patent**

**UNITED STATES PATENTS**

|           |            |               |
|-----------|------------|---------------|
| 2,463,264 | Graenacher | Mar. 1, 1949  |
| 2,483,392 | Meyer      | Oct. 4, 1949  |
| 2,488,094 | Graenacher | Nov. 15, 1949 |
| 2,515,173 | Ackermann  | July 18, 1950 |
| 2,604,454 | Ackermann  | July 22, 1952 |
| 2,785,133 | Craig      | Mar. 12, 1957 |

**FOREIGN PATENTS**

|    |         |               |              |
|----|---------|---------------|--------------|
| 75 | 611,510 | Great Britain | Nov. 1, 1948 |
|----|---------|---------------|--------------|